

## UNITED STATES PATENT OFFICE

2,247,876

ALLOY STEEL FOR THE MANUFACTURE OF  
WHEELS AND TIRESHarry L. Frevert, Philadelphia, Pa., assignor to  
The Midvale Company, Philadelphia, Pa., a cor-  
poration of DelawareNo Drawing. Application February 16, 1940,  
Serial No. 319,237

4 Claims. (Cl. 295—30)

My invention relates to alloy steel for the manufacture of locomotive tires, forged steel wheels and similar articles of manufacture which have to withstand the effects of heat, deformation and wear and which at the same time have to possess sufficient toughness or ductility to resist breakage due to sudden overloading or to stress concentrations.

Locomotive tires and forged wheels have been made for many years from plain carbon steel containing .5 to .8% of carbon, about the same percentage of manganese, silicon in amounts up to .30% and the usual very small percentage of impurities, particularly sulphur and phosphorus, common to steels of this type. Such tires and wheels have been subject, particularly under presentday conditions, to certain types of failure which have rendered them unfit for service or have necessitated frequent turning of the tread to produce the necessary service and life. The principal modes of failure have been by a shattering, spawling or "shelling" of the tread, by excessive wear or flow of the tread metal, or by "heat checking" that may result in breakage.

It has been found possible to retard failures of tires and wheels to some extent by heat treating them to increase strength and ductility prior to placing them in service. However, heat treatments, particularly those involving liquid quenching, unless carefully controlled, may produce defects difficult to detect by ordinary inspection and which eventually lead to complete failure. Furthermore, heat treating adds to the cost and its effects are sometimes nullified to more or less extent by the heating incident to shrinking of tires or other types of rings on the wheel centers.

Efforts have been made to improve tires and wheels by the use of alloy steels but the alloy contents have been so high or of such a character as to require that the finished article be also heat treated in order to attain the proper relationship between strength and ductility, the cost of the finished product then being much higher than that of heat treated plain carbon steel.

The object of my invention is to increase the service life of such wheels and tires by providing an alloy steel which, in respect to the qualities adapted to resist the types of failures above specified, more particularly hardness, tensile strength, ductility and toughness, is definitely superior to plain carbon steel. I accomplish this object by controlling the percentages of manganese and silicon and by adding, in such small percentages as not to add greatly to the cost, elements not present in carbon steel. My improved steel re-

quires no heat treatment. The cost of my improved steel does not, therefore, exceed, and if not heat-treated may be less than, the cost of heat treated plain carbon steel. In some cases, however, heat treatment of my improved steel will, as in the case of most steels, measurably improve it in respect of the qualities above named. However, in the absence of any treatment, other than those normally incident to the hot working of the article from the raw ingot form to the finished product, compositions embodying my invention possess properties sufficiently superior to those at present available in tires and wheels to make heat treatment unnecessary excepting in special cases. It will therefore be understood that my improved steel is capable of being produced on a competitive basis with plain carbon steel, which is one of the objects of my invention.

It will be understood that in the manufacture of carbon steel a fairly high degree (but often in degree less than is desirable) of hardness and strength is obtainable with sacrifice of toughness and ductility and that a fairly high degree of toughness and ductility is obtainable with sacrifice of hardness and strength, these qualities being controlled mainly by varying the percentage of carbon. For different uses primary consideration must be given to one or the other of these qualities. In my invention, also, both of these qualities are not obtainable in maximum degree in any single composition. My improved steel, however, is characterized by the fact that if its composition is so controlled as to be merely comparable with plain carbon steel having, for such steel, a high degree of hardness and strength, it greatly excels it in toughness and ductility, while if its composition is so controlled as to be merely comparable in toughness and ductility with plain carbon steel having, for such steel, a high degree of toughness and ductility, it greatly exceeds it in hardness and strength; as will be more fully understood by the comparisons made hereinafter. On the other hand, for most uses, where a high, but not maximum, degree of both specified qualities is desirable, my improved steel is characterized by these qualities to a degree hitherto unknown in plain carbon steel.

My improved steel contains carbon within a range known in plain carbon steels of this type, but to attain a given tensile strength, the percentage of carbon is distinctly lower. It contains manganese, within a range whose minimum is little, if any, below the maximum of the range usual in carbon steel. It contains, also, small percentages of chromium and molybdenum. The

addition of chromium alone has the effect of greatly increasing the strength but, if added in too large proportion, at too great a sacrifice of toughness. Its addition, therefore, must be in only a small percentage. With the addition of molybdenum in a very small percentage and with a carefully controlled increase in manganese, I have found that, after cooling from the hot working and forming operations, the desired increased hardness and strength are obtained without sacrifice of ductility and toughness.

The following are analyses of typical alloy steels embodying my invention.

|          | C       | Mn      | Si      | Cr      | Mo      |
|----------|---------|---------|---------|---------|---------|
|          | Percent | Percent | Percent | Percent | Percent |
| (a)----- | 0.64    | 0.92    | 0.10    | 0.36    | 0.08    |
| (b)----- | 0.72    | 1.00    | 0.28    | 0.43    | 0.10    |

It is of no substantial advantage to add any other element to the composition. Of course the usual amounts of sulfur and phosphorus, unavoidably present in steel, are contained, as impurities, in my composition, but if any other element is added it must be added in very small proportion and no element can be added that would impair the qualities characterizing my composition. As an example, an exceptional element that, when added in very small proportion, has no appreciable injurious effect and may have a slightly beneficial influence, is nickel, which, however, if present, should be held below .25%, since in greater amounts it tends to increase the air-hardening characteristics of the metal to too great an extent.

Tires, rings, wheels and forgings of this analysis forge and roll with the same facility as do plain carbon steels. The finished product is allowed to cool normally and uniformly in air.

The superiority of the above compositions to plain carbon steel will be appreciated by comparing them with the average properties found to characterize a large number of plain carbon steel locomotive tires such as are in everyday use.

|                                  | Tensile strength, lbs. per sq. in. | Elongation percent in 2" | Reduction of area, percent | Brinell hardness |
|----------------------------------|------------------------------------|--------------------------|----------------------------|------------------|
| (c) Plain .65% carbon steel----- | 122,500                            | 12.7                     | 20.8                       | 240              |
| Composition (a)-----             | 135,250                            | 13.0                     | 32.7                       | 270              |
| (d) Plain .75% carbon steel----- | 133,250                            | 9.8                      | 13.8                       | 266              |
| Composition (b)-----             | 152,400                            | 9.5                      | 23.1                       | 302              |

A comparison of composition (a) with composition (c) shows a pronounced improvement in strength and hardness, without impairment of, but on the contrary an improvement in, ductility and toughness. A comparison of composition (b) with composition (d) is equally favorable. On the other hand, a comparison of composition (a) with composition (d), which compositions are fairly comparable in hardness and strength, shows composition (a) to be greatly superior to composition (d) in ductility and toughness.

In producing plain carbon steel, where great hardness and strength for severe service are controlling, resort is had to high carbon, the upper limit of which, with the greatest practicable toleration of accompanying lower ductility, is about .75%. As our analyses show, the normal greatest tensile strength obtainable is about 133,000 pounds per square inch. In my improved steel

this degree of tensile strength is obtainable with carbon as low as .64%, without sacrifice of toughness and ductility in the smallest degree as compared with plain .64% carbon steel, which latter wholly fails to meet the specified requirements of hardness and strength. On the other hand, with a carbon content even lower than .75%, my improved steel has a tensile strength nearly 20,000 pounds per square inch higher than .75% plain carbon steel and without sacrifice of toughness and ductility and indeed with a substantial improvement in this quality.

The determination of the resistance to flow of my improved composition under load at elevated temperatures shows it to have properties in this respect far superior to those of ordinary carbon steel. Since the surface of railroad tires and wheel treads is subjected to heating while under load during service the improved resistance of the composition forming the subject matter of this invention to flow and consequent failure when heated is of considerable advantage in prolonging life in service.

It is clear, from the typical examples given, that the composition must be varied, although within narrow limits, to meet special requirements. Generally speaking, as in plain carbon steel, where hardness and strength are the primary requisites, the percentage of carbon is increased, while if the highest degree of ductility and toughness is required, the carbon percentage is lowered. It is desirable, also, with increase in carbon, to slightly increase the percentage of most, if not all, of the alloying elements. In all compositions embodying my improvement the carbon should always substantially exceed .50% and should rarely be lower than .60%, while it is undesirable that the carbon should exceed .75%, although in exceptional cases it may be increased to .80%. The percentage of manganese should never be lower than .70 or .75% and should not exceed 1.10%, although a percentage as high as 1.20 or 1.25% is exceptionally permissible.

Silicon should not exceed .40% and is preferably from .08 to .30 per cent. While chromium is indispensable, a very small percentage (not less, however, than .30 per cent.) will suffice. In most of my improved compositions .35 to .55% chromium is adequate. A higher percentage, but not over about .90 or (at the most) 1.00 per cent., is of advantage in exceptional compositions embodying my invention. Molybdenum, also, while indispensable, should not usually be in higher percentage than the chromium and should not usually exceed .30 per cent., although in exceptional cases it is advantageous to increase the percentage of molybdenum up to not over .7%. A percentage as low as .05% is sometimes adequate, although .10 to .15% is preferable.

In all compositions embodying my invention, the percentage of manganese substantially exceeds the combined percentage of any two of the other alloying ingredients (excluding carbon), while in compositions having in highest degree the characteristics hereinbefore described (illustrated by the specific compositions hereinbefore given) the percentage of manganese exceeds the combined percentage of all the other alloying elements (excluding carbon).

It will also be understood that the high carbon range herein specified is essential in the manufacture of tires, forged steel wheels and other articles, such as rings, roll sheets, sheave wheels and crushing machinery that require a certain degree of hardness and strength and that are sub-

ject to types of failures like or similar to those to which wheels and tires are subjected.

It will also be understood that the manufacture of wheel treads (by which term I intend to include treads integral with the wheels as well as wheel tires) has always presented a special problem, as hereinbefore explained, and that independently of the novelty of the composition per se, the discovery that such composition, as distinguished from an indefinite number of known alloy steel compositions, has superior resistance to the types of failure hereinbefore enumerated, which could be made only by making and testing the same, constitutes a new and useful improvement and a pronounced advance in the art.

What I claim and desire to protect by Letters Patent is:

1. Wheel treads and other ring-shaped articles of substantial thickness which are subject to types of failure that unfit them for service or unduly shorten their service life, composed of an alloy steel containing manganese between .70 and 1.25%, silicon between .05 and .40 per cent, chromium between .30 and 1.00% and molybdenum between .05 and .70%, the percentage of manganese being substantially in excess of the total percentage of any two of the other above specified alloying elements, and carbon over .50 and not over .80%, the balance of the composition being substantially iron, said articles, whether or not heat-treated, being characterized by superior wear hardness and strength without sacrifice of ductility and toughness and possessing superior resistance to said types of failure.

2. Wheel treads and other ring-shaped articles of substantial thickness which are subject to types of failure that unfit them for service or unduly shorten their service life, composed of an alloy steel containing manganese between .70 and 1.25%, silicon between .05 and .40%, chromium between .30 and 1.00% and molybdenum between .05 and .70%, the percentage of manganese being substantially in excess of the total percentage

of all the other above specified alloying elements, and carbon over .50 and not over .80%, the balance of the composition being substantially iron, said articles, whether or not heat-treated, being characterized by superior wear hardness and strength without sacrifice of ductility and toughness and possessing superior resistance to said types of failure.

3. Wheel treads and other ring-shaped articles of substantial thickness which are subject to types of failure that unfit them for service or unduly shorten their service life, composed of an alloy steel containing manganese between .80 and 1.10%, silicon between .08 and .30%, chromium between .30 and .55% and molybdenum between .05 and .15%, the percentage of manganese being substantially in excess of the total percentage of any two of the other above specified alloying elements, and carbon over .60 and not over .80%, the balance of the composition being substantially iron, said articles, whether or not heat-treated, being characterized by superior wear hardness and strength without sacrifice of ductility and toughness and possessing superior resistance to said types of failure.

4. Wheel treads and other ring-shaped articles of substantial thickness which are subject to types of failure that unfit them for service or unduly shorten their service life, composed of an alloy steel containing manganese between .80 and 1.10%, silicon between .08 and .30%, chromium between .30 and .55% and molybdenum between .05 and .15%, the percentage of manganese being substantially in excess of the total percentage of all of the other above specified alloying elements, and carbon over .60 and not over .80%, the balance of the composition being substantially iron, said articles, whether or not heat-treated, being characterized by superior wear hardness and strength without sacrifice of ductility and toughness and possessing superior resistance to said types of failure.

HARRY L. FREVERT.